

## UNITED STATES PATENT OFFICE

2,538,696

## LUBRICANT COMPOSITION

Robert L. May, Chicago, Ill., assignor to Sinclair  
Refining Company, New York, N. Y., a corpo-  
ration of Maine

No Drawing. Application August 23, 1946,  
Serial No. 692,705

3 Claims. (Cl. 252—46.6)

1

This invention relates to an improved mineral oil composition particularly useful as a heavy duty oil lubricant for internal combustion engines and having improved characteristics especially with respect to oxidation and corrosion and cleanliness of engine operation.

In my co-pending application Serial No. 545,193 filed July 15, 1944, of which the present application is in part a continuation, and which issued October 22, 1946, as Patent No. 2,409,877, there is described and claimed a mineral oil composition consisting essentially of a petroleum lubricating oil fraction and a minor proportion of an oxidation and corrosion inhibiting addition agent resulting from the reaction of an alkylated phenol with the condensation product of turpentine and phosphorus pentasulfide, the addition agent being more fully described and claimed in my Patent 2,379,312. For convenience, these addition agents are herein referred to as the oxidation and corrosion inhibitor or merely as the inhibitor.

In the above noted co-pending application I have also disclosed that the use of these inhibitors alone in proportions as great as about 1% of a 50% concentrate of the inhibitor or higher is subject to the disadvantage that there is a tendency toward sludging, due to excess phosphorus acidity, and that where such proportions of the inhibitor are used the effectiveness of the oil composition as an internal combustion engine lubricant is materially improved by the inclusion in the oil composition of a minor proportion of a so-called detergent consisting of an organic salt, or soap, of a metal capable of neutralizing the phosphorus acidity of the above noted oxidation and corrosion inhibitor.

The present invention is directed particularly to my improved mineral oil composition containing such detergent in conjunction with the oxidation and corrosion inhibitor of my said co-pending application, and provides means whereby the inhibitor may be used in proportions in excess of 0.5% by weight without experiencing difficulty due to excess phosphorus acidity.

Various organic salts and soaps have been found materially to improve the cleanliness of operation of internal combustion engines, when added in relatively small proportions to the lubricating oil used in such engines, and have been used for this purpose and commonly designated detergents. Notably among such detergents are the calcium, sodium and barium petroleum sulfonates, various calcium salicylates, especially calcium octyl salicylates, barium phenolate of sul-

2

furized diethyl phenol, calcium and barium phenolates of sulphurized tertiary amyl phenol, respectively, calcium soaps of oxidized lubricating oil acids such as that currently marketed in admixture with oil and containing about 1.75% calcium, and calcium ortho-lauroyl cresolate, described in Patent 2,307,615 to Barth.

These detergents have been found to be effective in inhibiting oxidation of the mineral oil with which they are admixed, over a substantial period of time, commonly designated the oxidation induction period. However, at the end of the oxidation induction period, these detergents appear to exert a prooxidant effect on the oil.

15 I have discovered that by the use of a detergent of the class noted in conjunction with the oxidation and corrosion inhibitor of my Patent No. 2,409,877 the disadvantageous tendencies of each of these materials when used alone are materially minimized. When so used together these materials have been found to be compatible, each accomplishing its intended purpose without destroying the effectiveness of the other. But, in addition, these two classes of additives have been 20 found to complement each other in such a way that excess phosphorus acidity of the inhibitor is effectively neutralized by the detergent, thus minimizing any tendency of the former to promote sludge formation, especially when the inhibitor is present in proportion as great as 0.5% or greater. Further the tendency of the detergent to promote oxidation of the oil at the termination of the oxidation induction period is also minimized by the presence of the inhibitor.

30 The proportions of the inhibitor and of the detergent used in the compounding of my improved mineral oil composition may be varied somewhat but in each case only a minor proportion of each is used. The proportion of the inhibitor is advantageous in excess of 0.5% by weight and may be as high as about 2.5% depending upon the amount and basicity of the detergent used. The detergent should be used in an amount at least sufficient to neutralize excess phosphorus acidity.

35 The optimum proportion to be used will vary somewhat with the particular inhibitor and detergent used and the intended use of the oil composition.

The oxidation and induction inhibitor is usually prepared as a 50% concentrate in a petroleum lubricating oil fraction, as hereinafter more fully described. The optimum ratio of the amount of detergent to the amount of inhibitor used will depend to a considerable extent on the basicity of the detergent and upon the amount of  $P_2S_5$

equivalent used in the preparation of the inhibitor and may be determined to any particular set of conditions by simple test. Usually the proportion of the inhibitor should not exceed that which will be neutralized by the detergent, as previously noted.

Various petroleum lubricating oil fractions may be used as the mineral oil constituent, for instance, Acid Treated Coastal Oil SAE 40, Acid Treated Mid-Continent Oil SAE 10, Solvent Treated Mid-Continent Oil SAE 30 or blends of such oils with bright stock or a solvent refined lubricating oil fraction from a Pennsylvania crude.

The invention will be hereinafter illustrated by specific examples of my improved mineral oil compositions. Since the characteristics of the inhibitor are somewhat affected by the characteristics of the turpentine-P<sub>2</sub>S<sub>5</sub> condensation product used in its preparation and the nature and proportion of the alkylated phenol reacted therewith, the illustrations of my lubricating oil composition will include a description of the preparation of the particular inhibitor used.

In the preparation of the intermediate turpentine-P<sub>2</sub>S<sub>5</sub> condensation product to be used in preparing my inhibitor, the molar ratio of turpentine to P<sub>2</sub>S<sub>5</sub> used is with advantage approximately 3:1 though this ratio may be varied somewhat as subsequently described.

The reaction of turpentine with P<sub>2</sub>S<sub>5</sub> is highly exothermic and proceeds spontaneously after being initiated by slight heating. A desirable method of effecting the reaction is to heat the turpentine in a vessel to about 200° F. or slightly higher and then, without further heating, slowly stirring in the phosphorus pentasulfide in the powdered form. The heat of reaction is great and, consequently, the addition should be made slowly, so as to avoid the possibility of the reaction's becoming uncontrollable. The characteristics of the inhibitor are favorably affected by using in its preparation a turpentine-P<sub>2</sub>S<sub>5</sub> condensation product in the preparation of which the temperature during the mixing was not permitted to exceed about 250° F., although higher temperatures are permissible.

After the addition is completed, it is usually necessary to apply heat externally to complete the reaction. The temperature during this last stage is preferably maintained at about 300° F., though temperatures of about 200° F. to 400° F. may be employed. This second stage of the operation should be continued until all of the P<sub>2</sub>S<sub>5</sub> is dissolved. The material thus prepared is a viscous liquid at elevated temperatures which solidifies on cooling to room temperature.

The turpentine-P<sub>2</sub>S<sub>5</sub> concentration products, thus prepared, are, in the absence of excess turpentine, brittle, resinous solids which dissolve readily in lubricating oils or in excess turpentine to form liquids. Such solutions of high concentration are relatively viscous. However, the viscosity of the solution decreases rapidly as the proportion of the solvent is increased from 25% to 75%.

In general, my inhibitor may be prepared by adding the alkylated phenol gradually to the turpentine-P<sub>2</sub>S<sub>5</sub> condensation product prepared as previously described. Such addition is advantageous at a temperature of about 230° F. However, this temperature may be varied, temperatures as high as 300° F. being used without damage to the product.

In reacting the alkylated phenol with the tur-

pentine-P<sub>2</sub>S<sub>5</sub> condensation product, very little heat is evolved. After the alkylated phenol has been added, the mixture is maintained at an elevated temperature, advantageously about 200° F. for about an hour with stirring. Satisfactory results have also been obtained where the alkylated phenol is added to the condensation product at a temperature of 275-280° F. and the mixture maintained at that temperature for about ten hours.

The proportions of the alkylated phenol may be varied over a considerable range without loss of the effectiveness of the resulting inhibitor. The optimum proportion of alkylated phenol used is, to a considerable extent, dependent upon the ratio of turpentine to P<sub>2</sub>S<sub>5</sub> used in the preparation of the intermediate condensation product. Particularly desirable results have been obtained using proportions of reactants equivalent to about 2 mols of P<sub>2</sub>S<sub>5</sub>, 6 mols of turpentine and 3 mols of alkylated phenol, assuming the molecular weight of turpentine to be 136. However, the proportions of these constituents may be varied somewhat. Satisfactory results may be obtained where for each two mols of P<sub>2</sub>S<sub>5</sub>, 5 to 8 mols of turpentine and 1 to 5 mols of the alkylated phenols are used. However, I have found it desirable that the total number of mols of turpentine and alkylated phenol used for each two mols of P<sub>2</sub>S<sub>5</sub> fall within a range of about 8 to 10. Also, in the preparation of the turpentine-P<sub>2</sub>S<sub>5</sub> condensation product used in preparing the inhibitor, I have found it desirable that no unreacted P<sub>2</sub>S<sub>5</sub> remain in the product.

In the preparation of my new class of inhibitors, considerable latitude is permissible in the selection of the alkylated phenol used. I have used with advantage alkylated phenols in which the alkyl radical of the alkylated phenol is a saturated aliphatic group, notably diaminophenol. However, other alkylated phenols may be used with advantage for instance, p-cyclohexylphenol, Pentaphen and the upper boiling petroleum cresylic acids. Each molecule of the alkylated phenol may contain one or more such groups. The number of carbon atoms in each aliphatic group is not critical. Desirable products may be obtained where each such group contains from 1 up to 12 to 16, or even up to 25 to 35 carbon atoms. Alkylated phenols containing 5 or more carbon atoms in each alkyl group have been found especially desirable in the preparation of my new inhibitors, because of the greater oil solubility of the resultant products. The alkyl group or groups may be either normal or branched chain.

Alkylated phenols, herein designated codimer alkylated phenols, such as prepared by the reaction, in the presence of sulfuric acid, of phenols with the olefines in commercial codimer, resulting from the phosphoric acid polymerization of mixed olefines of 4 carbon atoms or less per molecule and comprising propylene, butene-1, butene-2 and iso-butylene, the codimer consisting of a major portion of C<sub>3</sub> olefines, together with some C<sub>6</sub>, C<sub>7</sub>, C<sub>9</sub>, C<sub>10</sub>, C<sub>11</sub>, C<sub>12</sub> and higher olefines, have been used with advantage. These codimer alkylated phenols are comprised primarily of mono- and poly-alkylated phenols having alkyl groups, as noted above, but with C<sub>8</sub> alkyl groups predominating.

I have further used with advantage in the preparation of my improved inhibitors, alkylated phenols, herein designated codimer bottoms alkylated phenols, prepared by the method just de-

scribed for the preparation of codimer alkylated phenols except that the phenol was reacted with codimer bottoms, the codimer bottoms used being the bottoms obtained by a redistillation of the previously described codimer to a 350° to 360° F. end point overhead. This bottoms was comprised primarily of C<sub>12</sub> olefines, but contains some somewhat lower and some somewhat higher molecular weight olefines.

In the preparation of the turpentine-P<sub>2</sub>S<sub>5</sub> condensation product, either steam-distilled wood turpentine or gum spirits may be used. Such turpentine consists mainly of alpha pinene, a bi-cyclic terpene having the empirical formula C<sub>10</sub>H<sub>16</sub>. Pure alpha pinene and other more costly terpenes will react similarly with P<sub>2</sub>S<sub>5</sub>, but, for reasons including economic considerations, I generally prefer to use the more readily available turpentines. The turpentine used in the specific examples herein was a product known to the trade as "Pinene 111."

Various specific examples of these inhibitors and the details of their production are included in my Patent No. 2,409,877. In addition to those the following may be noted:

#### Example I

1,088 grams (8 mols) of Pinene 111 was placed in a 5 liter, three-necked flask equipped with a stirrer and thermometer and the temperature raised to 250° F. Then 444 grams (2 mols) of P<sub>2</sub>S<sub>5</sub> was added portionwise so as to maintain the temperature of the mixture between 250° to 275° F. this addition requiring 1 to 2 hours. After all of the P<sub>2</sub>S<sub>5</sub> had been added the mixture was heated for 7 hours at a temperature of 275° F. Thereafter 352 grams (2 mols) of p-cyclohexylphenol was added and the mixture heated an additional 4 hours at 275° F. When the resultant reaction was finished 2,045 grams of a petroleum lubricating oil fraction was added to reduce the viscosity of the product and reduce the percentage of the phosphorus pentasulfide in the resultant mixture to 11.3%. The mixture was then stirred an additional 30 minutes and was filtered while hot to give 3,929 grams of the final product. This product had an acid number of 12.2, a specific gravity of 0.9847 and contained 3.11% phosphorus and 8.41% sulfur.

#### Example II

The procedure followed in the preparation of this material was the same as that used in Example I except that 400 grams (2 mols) of upper boiling petroleum cresylic acids, having a boiling range of 247° to 298° C., was substituted for the p-cyclohexylphenol of the previous example, and only 1,997 grams of the mineral oil was added. The amount of the additive thus produced was also 3,929 grams. The acid number of the resultant product was 2.75, its specific gravity 0.9847 and it contained 3.13% phosphorus and 7.90% sulfur.

#### Example III

The procedure used in the preparation of this material was the same as that used in Example I except that 164 grams (1 mol) of Pentaphen was substituted for one mol of the p-cyclohexylphenol used in Example I and 2,057 grams of the mineral oil was added. The yield was 3,929 grams and the product had an acid number of 1.8, a specific gravity of 0.9868 and contained 3.22% phosphorus and 7.97% sulfur.

#### Example IV

This material was likewise made by the procedure of Example I except that 200 grams (1 mol) of the cresylic acids used in Example II was substituted for 1 mol of the p-cyclohexylphenol of Example I, and 2,021 grams of the mineral oil was added. The yield was 3,929 grams and the acid number of the product was 2.3. Its specific gravity was 0.9861 and it contained 3.05% phosphorus and 7.7% sulfur.

The effectiveness of my improved mineral oil composition as an internal combustion engine lubricant is illustrated by the following results of 36 hour engine tests using different detergents in conjunction with my inhibitor in various base oils.

In the following four tests, the base oil used was an acid treated Coastal Oil SAE 40 to which there was added 0.001% of a conventional foam inhibitor. The oil temperature in each case was 280° F.

Where neither inhibitor nor detergent was added to the base oil tested, the total varnish and sludge rating was 77, the bearing corrosion loss was 1.344 grams and analysis of the oil after the test showed an acid number of 1.5 and a viscosity rise of 219% at 100° F.

Where two parts of the inhibitor, such as produced in Example I, and 4 parts of calcium isooctyl salicylate were added for each 94 parts of the base oil, the total varnish and sludge rating was increased to 96.5, a very substantial improvement, the bearing loss was only 0.034 grams and analysis of the oil after the test showed an acid number of 0.5 and a viscosity rise of only 29.2%.

Where two parts of the same inhibitor and 16 parts of a solution of sodium mahogany sulfonate, consisting of 10 parts of the sulfonate and 90 parts of oil, were added for each 82 parts of the base oil, the total varnish and sludge rating was 82.5, the bearing corrosion loss was 0.140 gram and analysis of the oil after test showed an acid number of 1.4 and a viscosity rise of 66%.

Where 2.5 parts of the same inhibitor and 5 parts of a mixture of calcium soaps of oxidized lubricating oil acids in admixture with unoxidized lubricating oil and containing about 1.75% of calcium, previously identified, were added for each 92.5 parts of the base oil, the total varnish and sludge rating was 84.5, the bearing corrosion loss was 0.168 gram and analysis of the oil after the test shows an acid number of 2.8 and a viscosity rise of 113.1%.

In a similar test using as the base oil a solvent treated Mid-Continent SAE 30 oil the test of base oil alone, at an engine temperature of 265° F., showed a total varnish and sludge rating of 91, a bearing corrosion loss of 2.979 grams and analysis of the oil after the test showed an acid number of 2 and a viscosity rise of 48.4%.

Where 2.2 parts of the same inhibitor used in the preceding examples, 14.7 parts of calcium petroleum sulfonate, consisting of 10 parts of oil free calcium mahogany sulfonate in 90 parts of a lubricating oil fraction, 0.001 part of the foam inhibitor and 0.1 part of a conventional pour depresser were added for each 83 parts of the base oil, the total varnish and sludge rating was 96, the bearing corrosion loss was 0.059 gram and analysis of the oil after the test showed an acid number of 1.6 and a viscosity rise of only 17.7%.

A further oil subjected to this test, at an engine temperature of 265° F., consisted of 69.7 parts of an acid treated Mid-Continent SAE 10 base oil,

2.6 parts of the inhibitor, 26.4 parts of a 10% solution of oil free barium sulfonate in a neutral oil, 1.3 parts of a rust inhibitor and 0.2 part of the pour depresser. In this test the total varnish and sludge rating was 84.5, the bearing corrosion loss was only 0.082 gram and analysis of the oil after the test showed an acid number of 1.8 and a viscosity rise of 27.4%.

In each of the foregoing tests, with the exception of tests on the blank oil, the proportion of the inhibitor used was in excess of that which could be used in the absence of the detergent without evidence of a tendency toward sludge formation due to phosphorus acidity. By the inclusion of the detergent, this tendency was minimized as shown by the foregoing tests, in each instance the varnish sludge rating being in excess of that of the base oil in which the inhibitor was not included.

Further tests of base oils containing calcium ortholauroyl cresolate in conjunction with the inhibitors have shown a coke formation of only 0.06 gram where tests of the base oil alone showed 0.68 gram of coke.

A further advantage of my present invention, particularly as applied to solvent refined Mid-Continent and Pennsylvania Oils, is the clearness of the blend. It has been observed that when even relatively small proportions of the inhibitor, say of the order of 0.5%, are blended with such highly refined oils there is a tendency toward a slight haziness of the mixture. However, where a small amount of one of the herein described detergents is also present, up to 2.5 to 3% of the inhibitor may be added without causing noticeable haziness of the blend.

The method employed in determining the total varnish and sludge ratings, noted herein, is that described in the U. S. Army Tentative Specification AXS-1554.

I claim:

1. A mineral oil composition consisting essentially of a major portion of a petroleum lubri-

cating oil fraction, a minor proportion, effective to retard oxidation of the oil but not less than about 0.5%, of an inhibitor resulting from the reaction of an alkylated phenol with the condensation product of turpentine and phosphorus pentasulfide and a minor proportion effective to at least neutralize excess phosphorus acidity, of a detergent of the class consisting of calcium and barium petroleum sulfonates.

2. A mineral oil composition consisting essentially of a major proportion of a petroleum lubricating oil fraction, a minor proportion, effective to retard oxidation of the oil but not less than about 0.5%, of an inhibitor resulting from the reaction of an alkylated phenol with the condensation product of turpentine and phosphorus pentasulfide and in which excess phosphorus acidity is at least neutralized by the addition of barium petroleum sulfonate.

3. A mineral oil composition consisting essentially of a major proportion of a petroleum lubricating oil fraction, a minor proportion, effective to retard oxidation of the oil but not less than about 0.5%, of an inhibitor resulting from the reaction of an alkylated phenol with the condensation product of turpentine and phosphorus pentasulfide and in which excess phosphorus acidity is at least neutralized by the addition of calcium petroleum sulfonate.

ROBERT L. MAY.

#### REFERENCES CITED

The following references are of record in the file of this patent:

#### UNITED STATES PATENTS

| Number    | Name    | Date          |
|-----------|---------|---------------|
| 2,261,047 | Asseff  | Oct. 28, 1941 |
| 2,372,411 | Ván Ess | Mar. 27, 1945 |
| 2,409,877 | May     | Oct. 22, 1946 |
| 2,443,264 | Mikéška | June 15, 1948 |
| 2,486,188 | May     | Oct. 25, 1949 |